

Oct. 23, 1934.

S. C. LANGDON

1,977,639

METAL PROTECTED MIRROR

Filed Oct. 15, 1931

Fig. 1



Fig. 2



Inventor:  
SETH C. LANGDON

*Endicott*  
Atty.

## UNITED STATES PATENT OFFICE

1,977,639

## METAL PROTECTED MIRROR

Seth C. Langdon, Evanston, Ill., assignor to  
Curtis Lighting, Inc., Chicago, Ill., a corpora-  
tion of Illinois

Application October 15, 1931, Serial No. 568,899

6 Claims. (Cl. 88—1)

The present invention relates to metal backed reflectors, such as glass, particularly those which are used in connection with electric light bulbs for purposes of illumination, as in rooms, windows and like places, or electric arcs as in search lights and the like, or merely for ordinary mirrors.

Mirrors and reflectors have long been made using a silver film on the back of the glass as a reflecting surface. Pure silver has been employed for this purpose because it has an extremely high reflecting efficiency in the visible light range, and because methods of depositing the silver on the glass are well known and highly developed. To protect the silver film it has been a custom to deposit upon the silver film a covering coat of copper. This has been done largely and readily by depositing methods in a well known manner either chemical or electro-chemical. A protection is thus formed against injury by mechanical action and against corrosion of the silver by gases, and for conduction of heat away from the mirror.

The copper protected silver films have developed certain defects in usage. When the reflectors of copper coated silver are not in use, as when they are in storage, their life without defects is much greater than when the reflectors are in use for lighting purposes. In use they are subjected to the heat of the lamp or arc and this heat causes the defects to appear sooner. The defects may not always be of the same character. Sometimes the silver film is blistered. It may become dull and lose its sheen by the formation of a "blush" and there may be a mottling in areas of substantial size. Sometimes there is neither blistering nor blushing, nor mottling, but the surface loses its characteristic silver appearance, remains polished, but assumes a tinge of color more characteristic of copper than of silver.

The present invention is based upon the discovery of the cause of those defects, and it aims to improve upon the methods of protecting the silver to avoid the defects. It has been found by study that the copper in the protective coating and the silver of the film merge in some way sufficient to destroy the surface of the pure silver film at the junction with the glass. I have not determined whether the copper enters the silver coating without the silver entering the copper film, or whether one or both of the metals migrate from their original positions.

It has been noted that both silver and copper are analogous metals in many respects. They are both members of group I of the periodic system

of classification of the elements. In other words, they are so near alike in character and in properties that they readily merge together. The tendency exists, and, when conditions are favorable, as in the course of time, shortened by heat, they do mix. As a result of the mixing the color of the copper is imparted to the silver and a decrease in efficiency results.

The copper backed silver has many advantages, due in part, but not entirely, to the character of the backing being copper. The metal, whether copper or other metal, is a protective layer which is heat conductive. When the backing metal is thick compared to the film of reflective metal, it provides mechanical strength in addition to its protective action. Copper is easily plated onto a metal and in itself is cheap and economically applied.

The art heretofore has used relatively thick copper films plated onto silver reflecting films on glass in order to secure the protective and mechanical advantages thereby resulting. Such reflectors for heated lamps do not stand up in use. They are short lived, because of an interaction under the influence of heat between the thin silver film and the interface with copper. To avoid the cause of defects, and to preserve the advantages of copper backed silvered glass, I have made extensive studies and tests resulting in the present invention.

The general object of the present invention is to preserve all the advantages of a copper backed silver reflective film on glass and to eliminate all the inherent disadvantages.

A particular object is the formation of a metal partitioning film between the reflective film and a backing metal which backing is disadvantageous when directly united to the reflective metal, like copper on silver.

Another object of the invention is the use of a non-analogous metal such as metal from a different group in the periodic system of classifying the elements.

A particular object is the use of a partitioning film of a metal, or alloys of metals, from group VIII of the periodic system, including iron, nickel and cobalt.

A further object of the invention is the use of nickel between the silver and a backing metal.

Still another object is the use of copper on nickel on silver as a laminated metal coating on glass.

In the accompanying drawing:

Figure 1 shows a cross-section of a lamp reflector embodying the present invention.

85

90

100

110

Figure 2 shows an enlarged cross-section of the material of the reflector.

It will be understood that both curved and plane sections of reflector may embody the invention, and that any reflector may combine both curved and plane sections. The form, size and shape of the reflector illustrated in the drawing is by no means intended as a limitation of the invention to that form or to the particular use illustrated.

The preferred embodiment of the invention is briefly described, but without intention to limit the invention thereto. The preferred embodiment merely illustrates the nature of the invention. The scope of the invention may be readily understood from the discussion which follows the detailed reference to the drawing.

A lamp 10 of the incandescent type is illustrative of a light which is incidentally a source of heat. An arc light might also be employed or a neon tube may be used. The numeral 11 designates a suitable reflector, which is here designed and constructed for use with the bulb type of electric lamp 10. The reflector is made of transparent glass indicated at 11. A reflective metal, such as silver 12, is deposited on the glass in a film of sufficient thickness to be a suitable silver reflecting film, as is well known in the art. Onto the silver film a thin metal film is deposited, preferably by electro-plating a metal such as nickel 13, or its functional equivalent, but not copper or its functional equivalent. The nature of equivalency is to be measured in terms of disclosures hereinafter made, and is not to be considered as a generality involving properties not material to this invention. Onto this partitioning metal there is deposited, preferably by electroplating, a thick film of mechanically functioning metal, such as copper 14, or its functional equivalent.

Because the bare external copper film does not present an attractive appearance, I may add a finishing composition. I prefer to use one which is functional to emit heat rapidly from the heated reflector. A coating may be employed which acts as an insulator, but this causes the working temperature of the reflector in use to be higher. I employ a coating which has a high power of emissivity. Numerous emissive surfaces may be employed and these are described in my copending application, Serial No. 591,107, filed Feb. 5, 1932. I prefer to use an enamel type, such as a synthetic resin varnish which may be baked on, containing ultimately from 10% to 80%, more or less, of a bronze metal powder, such as the bronzes made by surface oxidation of powdered copper metal or alloys of copper. The coating generally is designated at 15, the bronze particles at 16 and the matrix therefor at 17. The reflector so made with this enamel is commercially advantageous because of the present invention.

Having discovered that heat accelerates the injury to a silver film when backed with copper, I aim to reduce any similar action between the reflective film and a backing metal, by lowering the working temperature of the reflector. One way to do this is by metal backings of high thermal conductivity. Another way is by increasing the emissivity of the non-reflecting surface of the reflector. I also employ a metal next to the reflective metal which is very little affected by the conditions which affect copper. Where I desire copper as a metal in the reflector I place between the copper and the reflective metal, a metal less reactive with silver than is copper, such as nickel

on reflective silver. It acts as a partition and only a relatively thin coating is necessary to isolate the copper and the silver.

I have determined that a nickel film of about 60 atoms of thickness is much thicker than is required for commercial purposes and that a layer 1200 atoms thick is quite suitable. In practice, however, it appears to be more difficult and expensive to control the thickness of the layer to such a fine degree as above mentioned, than to form a much thicker coating. In special tests with thickness of varying degree I have found that the life is prolonged as the thickness of nickel increases. It is only necessary to place sufficient nickel or its equivalent onto the silver to secure a desirable commercial life for a given working temperature.

For example I have made measurements and calculations which are herein given to illustrate the order of thickness and the relative thicknesses of the respective layers. The measurements made are not to be considered as absolute, nor reproducible, and it is to be understood that the conditions of deposition may control the density of the deposited metals.

| Metal       | Atoms thick | Millimeters thick | Inches thick | Rates (silver=1) |
|-------------|-------------|-------------------|--------------|------------------|
| Silver..... | 1300        | .000055           | .000022      | 1                |
| Nickel..... | 1200        | .00033            | .0000133     | .6               |
| Copper..... | .005        | .002              |              | 9                |

Nickel, cobalt and iron, either alone or in alloyed form, are all good partition agents for copper and silver. Other metals non-analogous to silver may be used, and the more remote they are, as determined by their position in the periodic system, the better suited they are.

The metals of group VIII are the most practical so far as I am able to determine. Lead is too close to silver and it easily alloys. Lead is in group IV, and silver in group I, which groups are separated by only two other groups. I therefore believe that the metals should lie in groups separated by at least three other groups. However, I prefer the ferromagnetic group of metals as the group for selecting the partition agents. Metals within groups V to VIII may be considered as equivalents of nickel for use adjacent silver, but many of them may be impracticable.

The following examples show suitable methods which may be used for depositing the partitioning metal or alloy onto silver:

As a basis for depositing the coating any silvered reflector may be employed which presents at the non-reflecting surface a silver metal area to which the protective coating may be metallically united. Such silver films may be deposited in any well known manner of which the preferred form is the application by silver solutions containing chemical reducing agents which effect decomposition of the silver compound in solution to deposit the reflecting silver film on the glass or other medium.

*Example 1, iron.*—To deposit iron on such a silver film the following solution may be employed:

|                                                    | Grams |
|----------------------------------------------------|-------|
| Ferrous chloride (dried) (FeCl <sub>2</sub> )..... | 190   |
| Calcium chloride (dried) (CaCl <sub>2</sub> )..... | 250   |
| Water to make a solution of 750 cubic centimeters  | 145   |

The solution is used as an electroplating bath with an anode of iron, using the silver film as

silver in the prior art. By eliminating the sensitive reactive interface with silver, I may employ the thermal property of copper to an advantage to the new interface. Thus the new interface and 5 copper cooperate with each other to prolong the life of the reflector.

In manufacture of reflectors of this invention, and in the manufacture of reflectors of the prior art it has been a custom to bake onto them a 10 finishing enamel. It is of course not essential. But in the process of baking a copper-coated silver, the baking heat helps to start the destructive reaction in the reflector before its process of manufacture is complete. When the substitute and 15 more stable interface is used the reaction takes place much slower and without injury to the life of the reflector.

The invention therefore has several aspects. In one view, it comprises a metal backed silvered 20 glass in which the metal, such as copper, is separated from the silver by a metal which is less reactive towards silver. In another view, it comprises a silvered glass covered with two layers of 25 united metals, the outer one being more conductive of heat than the metal adjacent the silver.

It is to be understood that the partitioning layer 30 may be an alloy, such as those hereinabove described, and also that the strengthening layer may be an alloy, as well as being copper. The word "metal" is not limited in meaning to elemental metal, but includes an alloy of elemental metals.

In the accompanying claims I am to define the invention as including the preferred form and the modifications or changes from the preferred 35 form which are dictated by this disclosure and by the two related aspects of the invention as above set forth.

What I claim is:

1. A light reflector adapted to withstand heat 40 comprising a glass reflector body, a reflective film of silver on said body, a film of nickel metallically united to the silver, and a layer of copper metallically united to the nickel.

2. A light reflector adapted to withstand heat 45 comprising a glass reflector body, a reflective film of silver on said body, a film of nickel metallically united to said silver on said body, and a

layer of metal more conductive of heat than is nickel metallically united to the nickel.

3. A light reflector adapted to withstand heat comprising a glass reflector body, a reflective film of silver on said body, a layer of metal chosen from the ferro-magnetic group including iron, nickel and cobalt, said layer being metallically united to the silver, and a third layer of metal metallically united to the second layer, said third layer being of metal more conductive of heat than 80 the second layer. 85

4. A light reflector adapted to withstand heat comprising a glass reflector body, a reflective film of silver on said body, a layer of metal chosen from the ferro-magnetic group including iron, nickel and cobalt, said layer being metallically united to the silver, and a third layer of copper 90 metallically united to the second layer.

5. A light reflector adapted to withstand heat comprising a glass reflector body, a reflective film of silver on said body, a layer of metal chosen from the ferro-magnetic group including iron, nickel and cobalt, said layer being metallically united to the silver, and a third layer of metal 95 mechanically united to the second layer and 100 thicker than said second layer whereby to provide mechanical strength.

6. A light reflector designed and adapted for use in proximity to a source of light which is also a generator of heat, comprising a mirror located 105 in heat-receiving proximity to said source of light, such mirror comprising a transparent element facing said source of light, an opaque reflective layer of silver closely adherent on the side of said transparent element away from said source 110 of light, a second opaque layer of metal upon the side of said reflective silver layer away from the source of light, which second layer of metal is selected from a group of metals consisting of 115 iron, nickel, cobalt, (the substantially silver-coloured alloys of such metals), chromium and platinum, and a third layer of metal metallically united to said second layer, and having a higher degree of heat conductivity than has the metal of said second layer. 120

SETH C. LANGDON.

50

125

55

130

60

135

65

140

70

145

75

150